

# UNITED STATES PATENT OFFICE.

ERNEST BATEMAN, OF MADISON, WISCONSIN.

## METHOD OF BLEACHING WOOD.

1,329,284.

Specification of Letters Patent.

Patented Jan. 27, 1920.

No Drawing.

Application filed September 8, 1919. Serial No. 322,580.

(FILED UNDER THE ACT OF MARCH 3, 1883, 22 STAT. L., 625.)

*To all whom it may concern:*

Be it known that I, ERNEST BATEMAN, an employee of the Department of Agriculture, residing at Madison, Wisconsin, (whose 5 post-office address is Madison, Wisconsin,) have invented a new and useful Method of Bleaching Wood.

This application is made under the act of March 3, 1883, chapter 143 (22 Stat. 625), 10 and the invention herein described and claimed may be used by the Government of the United States or any of its officers and employees in the prosecution of work for the Government of the United States or any 15 of its officers and employees in the prosecution of work for the Government and any person in the United States without payment to me of any royalty thereon.

In the manufacture of chairs and other 20 furniture from oak or other woods where a light color is desired, it frequently happens that considerable difficulty is encountered in matching the various sections so as to produce a uniform color or shade which is essential in the best types of office furniture. 25 Moreover, when the sections are matched as nearly as possible before manufacture, in the process of manufacture one or more of the sections becomes darker during the process, 30 with detrimental results to the finished products. This is particularly so if any section is steamed and bent during the process.

I have discovered that by the use of a solution containing nitric acid and a chlorate, 35 such as potassium or sodium, a lighter and more uniform color is obtained, and when the solution is properly applied to sound wood the strength of the wood is not materially affected. The concentration of the 40 nitric acid and chlorate salt may vary with-

in rather wide limits, depending somewhat on the nature of the work, the time in which the bleaching must be obtained, and the shade or color desired. Where brilliant shades of yellow are desired, I prefer to use 45 a solution of concentrated nitric acid which has been saturated with potassium or sodium chlorate. This solution is allowed to act for only a short length of time. Where less brilliant yellows are desired, I prefer to 50 use a mixture of concentrated nitric acid saturated with potassium chlorate and diluted with an equal volume of water; the wood being subjected in this case to a somewhat longer treatment than in the previous 55 solution. Where pale yellows are desired, I prefer to use a saturated solution of potassium chlorate mixed with one-third its volume of concentrated nitric acid. In the practice of my invention I apply the solution prepared as above described to the wood 60 in any suitable manner. The wood may be dipped in the solution, or the solution may be spread on the surface of the wood by means of a suitable brush. I then dry the 65 material as quickly as possible in a heated oven.

I claim:

A method of bleaching wood which comprises applying thereto a solution of concentrated nitric acid combined with potassium chlorate. 70

In testimony whereof, I affix my signature on this 11th day of August, 1919, in the presence of two subscribing witnesses.

ERNEST BATEMAN.

Witnesses:

L. F. HAWLEY,  
S. A. MAHOD.